

Nov. 1, 1932.

A. MEISSNER

1,886,235

METHOD OF STABILIZING NONCRYSTALLINE PIEZO ELECTRIC MICROPHONE DIAPHRAGMS

Filed Sept. 10, 1929

*Fig. 1*



*Fig. 2*



INVENTOR  
ALEXANDER MEISSNER  
BY *H. G. Love*  
ATTORNEY

## UNITED STATES PATENT OFFICE

ALEXANDER MEISSNER, OF BERLIN, GERMANY, ASSIGNOR TO TELEFUNKEN GESELLSCHAFT FÜR DRAHTLOSE TELEGRAPHIE M. B. H., OF BERLIN, GERMANY, A CORPORATION OF GERMANY

METHOD OF STABILIZING NONCRYSTALLINE PIEZO-ELECTRIC MICROPHONE DIAPHRAGMS

Application filed September 10, 1929, Serial No. 391,585, and in Germany August 1, 1928.

This invention relates to the piezo-electric art and deals more specifically with the production of piezo-electric materials from non-crystalline substances.

In accordance with the principles of this invention it has been found experimentally that if such materials as resins, waxes, asphaltum, or the like, are heated and then allowed to cool, direct current potential being applied to the body during cooling, the resulting material exhibits good piezo-electric properties and may be utilized in high grade microphones or in other cases where the present day crystalline piezo-electric materials are used.

It has also been found, in accordance with the principles of this invention, that the piezo-electric properties of the body thus produced may be substantially increased by the addition of a powdered piezo-electric body such as quartz, for example.

The manner in which the present invention is carried out will be more clearly understood from the following description taken in connection with the accompanying drawing in which:

Fig. 1 is a diagrammatic view showing a system embodying the principles of the present invention; and

Fig. 2 is a diagrammatic showing of the properties of piezo-electric elements in accordance with the principles of this invention.

Referring in detail to Fig. 1, a piezo-electric plate or diaphragm P is connected to the input circuit of a vacuum tube amplifier R. It will be understood that the present figure discloses, by way of example, the use of the piezo-electric element as a microphone. Obviously, the piezo-electric body may be used, in accordance with the principles of the present disclosure, for all purposes for which piezo-electric bodies are now used, such as, for example, as a means to maintain constant the frequency of an oscillation generator, a frequency standard, or other uses.

It has been found, in accordance with the principles of this invention, that a piezo-electric body of the type herein disclosed loses its piezo-electric action or moment in the

course of time but that such decrease in piezo-electric action can be either entirely eliminate or retarded to a substantial degree by applying across the terminals of the piezo-electric body a direct current potential. In the figure the direct current source B is shown permanently connected to the terminals of the crystal P. In order not to impair the operation of the vacuum tube R a blocking condenser C is applied between the grid of the vacuum tube and one terminal of the crystal, thus cutting off the direct current potential between the filament and grid of the vacuum tube R.

The condenser C is proportioned so that the alternating current potentials, created when the plate or diaphragm P responds to voice waves, are allowed to act upon the grid of the tube R in a manner well understood.

It is important, in accordance with this invention, that the battery potential B be applied to the plate P in the proper direction, that is, the polarity of the battery must be properly chosen with respect to the plate. In this connection, it has been discovered that for some materials, for instance, sealing wax, the piezo-electric action will always maintain the identical sign. In other words, the piezo-electric action corresponds to the potential which was applied to the plate when the latter was being formed. Hence, in order to preserve and maintain the piezo-electric action the potential furnished from battery B must be of the same sign or sense of flow as was the former potential. Other substances, such as electret, asphaltum, etc., whether with or without an addition of powdered quartz, exhibit the peculiar property that immediately after forming they exhibit the piezo-electric action or moment in the same sense as the source of forming potential.

After a few days the value of this moment drops to zero. Thereafter, however, it grows again but in the opposite direction and the permanent condition finally is that the plate exhibits a moment having the opposite sign as compared with that which it had immediately after the discontinuance of the forming process. Fig. 2 shows graphically the variation of the piezo-electric moment for sub-

stances of this kind plotted against the time.

In the technical press it has become customary to designate a substance of a special nature in which the permanent electric moment is preserved through years, as "electret".

5 This substance has been more exhaustively investigated by M. Eguchi, Phil. Mag., 49, 1925, p. 178, and it consists of a mixture of 45% colophony, 45% carnauba wax and 10% beeswax. This special material having a 10 composition as just indicated is meant in the present application as "electret". The property of the latter to carry permanent electric momentums, as can be seen from the application, is possessed by a number of other substances, for instance, different kinds of resins, waxes, sealing wax and asphaltum.

It has been found, also, that this final state, after the reversal of polarity, in some materials decreases gradually but that the positive maximum of the moment is slightly greater than the moment in the negative direction. It therefore becomes desirable to provide an arrangement which is adapted to maintain this positive maximum of the piezoelectric action. To accomplish this result it has been found advisable to apply a direct current potential after the forming process of a plate though in the opposite sense as compared to the potential applied before.

20 30 It will be understood that various changes in the specific embodiments disclosed herein will readily suggest themselves to those skilled in the art and the present invention, therefore, is not to be limited except as defined in the appended claims.

Having thus described my invention, what I claim is:

1. A piezo-electric element comprising a 40 body of the class of materials including resins, waxes, asphaltum and electret.

2. A piezo-electric element comprising a body of the class of materials including resins, waxes, asphaltum and electret in combination 45 with quartz.

3. A piezo-electric element comprising a body of the class of materials including resins, waxes, asphaltum and electret in combination with powdered quartz.

4. In combination, a piezo-electric body 50 and means to maintain said body piezo-electrically active, said means comprising a source of direct current potential connected to said body.

5. In the method of preparing a piezo-electric body, the steps of heating the material from which said body is to be formed, permitting said body to cool and maintaining a direct current potential upon said body 55 during the cooling operation.

6. A method of stabilizing a non-crystalline body possessing piezo-electric properties which comprises applying a unidirectional potential to the electrodes of said body.

65 7. Method according to claim 6, character-

ized in that the potential is applied immediately after forming the plate, and that the sense of said potential is the same as that of the forming potential.

8. Method according to claim 6, characterized in that the potential is only applied to the plate after a reversal in polarity has taken place in the plate subsequent to forming, and that the sense of said potential is opposite that of the potential used during the forming process.

9. In combination, an electron discharge device having a cathode, anode and control electrode, a non-crystalline piezo-electric body connected to said cathode and control electrode, a source of direct current potential located across the plates of said piezo-electric body, and a blocking condenser located intermediate said control electrode and said body.

ALEXANDER MEISSNER.

70

75

80

85

90

95

100

105

110

115

120

125

130